

May 2, 1933.

J. E. LILIENFELD

1,906,691

ELECTRICAL CONDENSER DEVICE

Filed March 28, 1928

Fig. 1.



Fig. 2.



Fig. 5.



Fig. 3.



Fig. 4.



Fig. 6.



INVENTOR

Julius Edgar Lilienfeld

BY  
Reinhard Schuetz  
ATTORNEY

## UNITED STATES PATENT OFFICE

JULIUS EDGAR LILIENFELD, OF BROOKLYN, NEW YORK

## ELECTRICAL CONDENSER DEVICE

Application filed March 28, 1928. Serial No. 265,373.

The invention relates to a condenser device for use in connection with electric circuits; and it has for its object the provision of a simple, compact, substantial and effective 5 device of this character which while shall be comparatively inexpensive to construct; also, a condenser which shall have extremely high specific capacity—of the order of magnitude of 0.02 mfd. per  $\text{cm}^2$ , with a total 10 thickness of the finished product which may be less than 1 mm.

If a coating of compounds of a metal, for example, the oxide of aluminum, magnesium, tantalum, tungsten, etc., be produced 15 partly or entirely over a surface of the respective metal selected, or an alloy of several of these metals, an insulating layer having high dielectric properties may be attained; and I have discovered that such layers may 20 be used in a minute thickness as the dielectric of a commercial condenser, provided a further layer or coating of substantially more conductive material be integrally associated therewith by applying this material 25 in disintegrated or finely subdivided state, e. g. by spraying or by spattering it in a vacuum cathodically from such metals as copper, lead, aluminum, etc., over said dielectric layer. Or said layer may be applied 30 by colloidal precipitation, it being understood that substantially molecular contact over the whole area is had between it and the dielectric layer. Under these circumstances such insulating layers, I also have 35 discovered, do not possess rectifying properties similar to those which are being shown by different combinations, for example, when aluminum oxide is deposited on an aluminum electrode of an electrolytic cell with ammonium borate as electrolyte; on the contrary, the layers show insulating properties for 40 voltages applied in either direction.

The underlying or base material is preferably of relatively thin metal, approximately 0.03 mm. or less, to prevent, in case of bending, distortion of the same and injury to the superposed layers.

In some cases it may be advisable to apply 45 more than one coating over the first and insulating layer in succession in the manner

indicated, in order to increase the effectiveness of the insulation, a final coating of particularly good conducting quality, as of silver, platinum, tin, nickel, aluminum, etc., however, being generally provided so as to 55 secure a good contact for the outside lead. These coatings, in particular as well as in certain instances also the initial coatings, may be precipitated from colloidal metal suspensions; or they may be "metal-sprayed". 60

The dielectric layer or layers when thus coated maintain a highly insulating property, affording a substantial insulation between the underlying metal which represents one of the condenser plates and the conducting coating or coatings which represents the other plate of the condenser, so that it is possible to apply voltages of the order of magnitude of 100 volts across a dielectric 70 thus produced and of a thickness of the order of magnitude of only  $10^{-4}$  mm. without puncturing it. In fact, the condenser will in many instances possess self-healing properties. In an aluminum-aluminum oxide condenser 75 with an oxidizable conducting layer of copper, aluminum, magnesium, etc., short circuits will disappear as soon as the condenser is momentarily subjected to a load. This is a possible explanation of the fact, which I have discovered, that the allowable voltage 80 appears to be a function not only of the nature and thickness of the dielectric layer but also of the physical and chemical properties of the superposed coatings.

A coating produced by spattering from a 85 copper cathode over the dielectric layer, for example, imparts to the layer the property of withstanding a higher voltage than silver similarly applied. The more effective coatings, however, may, in some cases, not be very 90 highly conductive; and it is, therefore, sometimes desirable to provide more than one coating over the layer, the outer of them to possess a particularly good conducting quality; and the same may be applied in any suitable manner, for example, electrolytically.

The dielectric layer may readily be attained of said minute thickness by electrolytic 95 or by purely chemical methods, e. g. heat oxidation, sulfurization, etc., forming the same 100

of and directly on the metal base which represents one of the condenser plates; for example, a dielectric layer consisting of the oxide of aluminum thus formed directly of an underlying solid conducting base of aluminum has been found very satisfactory for this purpose. Over this layer is to be provided the superposed coating of substantially greater conductivity than the dielectric, and suitable provision is to be made for affording electrical connection on one hand with the base element and on the other hand with the conducting coating located about the intermediate dielectric.

15 In many cases, very satisfactory results are had with the superposed coating consisting partly or wholly of a compound of certain metals; and this may be attained in different ways. For instance, if a metal, e. g. copper, electrode is used in spattering, layers of different natures may be obtained according to the gas filling of the spattering container in which the spattering is conducted as well as to the electrical conditions prevailing therein. Thus, either a pure metallic layer, (Cu), layer of a compound (Cu<sub>2</sub>O) or, preferably, a mixture of both may be produced directly by the spattering process.

On the other hand, compounds particularly suitable for this purpose may be obtained by subjecting a spattered coating to subsequent chemical treatment. For example, the coating initially deposited may be treated in sulfur vapor or with carbon disulfide in which elemental sulfur is dissolved; or, it may be subjected to oxidation by heat treatment or by oxidizing reagents, e. g. H<sub>2</sub>O<sub>2</sub> etc.; or, it may be treated, as in the case of a coating of lead, in vacuo with atomic oxygen in order to convert it into PbO<sub>2</sub>.

A very compact and extremely effective condenser is attained in the aforesaid manner, it being possible to thus construct condensers of integral structure having a constant specific capacity which may be as high as 0.02 mfds. per cm<sup>2</sup>. more or less, according as the polarizing voltage in the preparation of the underlying or base material was low or high, while the total thickness of the commercial product may be substantially less than one millimeter, depending on the materials used.

In the accompanying drawing which illustrates the invention:

55 Fig. 1 is a fragmentary longitudinal section illustrating the novel condenser and shown greatly magnified and on a disproportionate scale for purpose of illustration.

Fig. 2 is a similar view illustrating a modification.

Figs. 3 and 4 are respectively a front elevation and transverse vertical section of a completed condenser unit, but shown greatly magnified and on a disproportionate scale for purpose of illustration.

Figs. 5 and 6 are similar views illustrating a further embodiment of the condenser, Fig. 5 being a front elevation and Fig. 6 a horizontal section taken on the line 6—6, Fig. 5.

Referring to the drawing, 10 designates a metal such as aluminum, magnesium, tantalum, tungsten, etc., which forms the base or supporting element of the condenser; and, in accordance with the invention, there is provided over a portion of the surface thereof, 70 or over substantially the entire surface if desired, a non-conducting or insulating layer 11 which is formed as a compound of the particular metal forming the said base member. For example, if aluminum be selected 80 as the base member, the insulating layer 11 will be the oxide of aluminum (Al<sub>2</sub>O<sub>3</sub>), which may be provided thereon in any suitable and well-known manner as by electrolytic or purely chemical methods. If, in the 85 former instance, a high voltage condenser is to be formed, it is advisable to employ voltages as high as possible; and when aluminum is utilized as the base material, the voltage in the electrolytic process will range 90 up to 400 volts in an aqueous solution and up to 1,500 volts in an alcoholic solution. This layer then is an integral part of the base material which is selected, also, to be of relatively thin stock—approximating 0.03 mm. or less, 95 so that in case of bending of a completed condenser unit there will be no serious distortion of the said base member and resulting injury to said layer of oxide, as well as to the further coatings hereinafter more fully set 100 forth. The dielectric layer itself is to be of minute thickness only, for example, of the order of magnitude of 10<sup>-4</sup> mm., so as to afford the extraordinarily high specific capacities attained when provided with a 105 superposed substantially more conductive coating or coatings integrally associated therewith.

To this end, there is provided over the aforesaid layer of oxide and in a molecular 110 contact with it over the total contact area one or more substantially more conductive coatings 12 and 13 of disintegrated or finely subdivided metal or metallic compounds, or mixtures of such metal and compound. 115

These coatings may also be of extreme thinness, in fact not any thicker than required in order to provide for a good contact possibility, and are applied in disintegrated or finely subdivided state, as by spattering 120 cathodically from such metals as copper, lead, aluminum, etc., the desired coatings. Or, the same may be attained by precipitation from colloidal metal suspensions or by pressure spraying. A purely metallic coating or a 125 coating consisting of a metal and compound thereof, or solely a compound, may constitute the layer 12, for example, as a copper and copper oxide mixture.

However, while such coatings of mixtures 130

or solely compounds appear to be capable of increasing substantially the upper limit of the allowable voltages some of them are not very highly conductive; and it may be advantageous in particular cases to provide thereover an additional coating 13 of particularly good conducting quality, as well as having nontarnishing properties, for example, a coating of silver, nickel, aluminium, etc.

10 Compounds especially suitable for the purpose of increasing the puncturing voltage may be obtained by a subsequent treatment of the deposited coating as by treatment in sulfur vapor or with carbon disulfide in which elemental sulfur has been dissolved. Or, a deposited coating may be subjected to oxidation by heat treatment or by means of oxidizing reagents such as  $H_2O_2$ , etc.; or in vacuo with atomic oxygen as in the case of 20 a coating of lead in order to convert it into  $PbO_2$ . In Fig. 2 a condenser thus constituted is indicated, the outer and final coating 12 overlying the dielectric layer of aluminum oxide consisting of copper sulfide ( $Cu_2S$ ).

25 In Figs. 3 and 4, a practical embodiment of the invention has been set forth, the same comprising a centrally disposed base element 15, as of aluminum, upon which has been provided a layer 16 of aluminum oxide, as aforesaid, the same in this instance substantially covering the entire surface of the base element 15 with the exception of a projecting tongue member 17 thereof. Two further coatings 18 and 19 are applied over 35 the said oxide layer, the under coating consisting of a mixture of copper and copper oxide while the outer consists of silver.

Contact with the condenser thus afforded 40 may be through a pliable conducting material such as tin or lead foil 20 which insures a good contact with the outermost coating 19 and affords, also, ready means for outside connection as through a conductor 21 attached thereto. Further contact may be 45 had to the condenser through the tongue 17, as through a conductor 22, thus completing the means for applying voltage to said condenser. Moreover, an insulating cover 23

50 as of varnish, paper, rubber, etc., is provided over the tongue 17 and portion of the foil 20 to prevent short-circuiting of the condenser elements. The condenser thus constructed may be placed in an air-tight envelope or the 55 like (not shown) and suitably protected in accordance with the usual practice.

While the design of condenser indicated in Figs. 3 and 4 has been found satisfactory for lower voltages, it is advisable to modify 60 this design somewhat when the condenser is to be utilized in connection with high voltages and more particularly to the extent of avoiding contact of the underlying oxide-coated aluminum base element 15 and 65 the contact-making surrounding foil 20 with

the edges of the overlying more conductive coating or coatings 18 and 19.

In order to satisfy this condition, reference being had to Figs. 5 and 6 of the drawing, the base element 25 is completely oxide-coated as in the previously described embodiment, but the overlying substantially more conductive coating 26 is applied in a manner to leave a margin of the oxide layer entirely surrounding said coating 26. Over the latter is then arranged a strip of insulating paper 27, or the same may be wrapped around the base with coating, said paper being provided with a window or windows 28 slightly smaller than the conducting coating so as to overlap the outline of said coating. Over the window or windows is then placed or wrapped a layer of tin foil 29 or the like to enclose the condenser except for the projecting tongue member 30 thereof, the foil being pressed inwardly through the corresponding window so as to afford a contact to the conducting coating 26.

The novel condenser herein set forth has been found capable of withstanding applied voltages of the order of magnitude of 100 volts with a dielectric or insulating layer, as the layer 16, of an order of magnitude of only  $10^{-4}$  mm.; and a very compact and effective device is thereby afforded, it being found possible to construct condensers of this type of a capacity as high as 0.02 mfd. per  $cm^2$ . while the total thickness of the commercial condenser need not be over 1 mm. and may be substantially less, depending upon the materials utilized. Through the contacts or terminals provided as aforesaid, a number of the novel condenser units may be interconnected in parallel or series relationship, or both, and in manner well understood, to provide for various combinations of capacities and voltages required. While the dielectric insulates, of course, in either direction of current flow, it has been found preferable to connect the positive (+) potential to the aluminum or underlying base element of the condenser in the case of the application of direct current thereto.

I claim:

1. An electrical condenser, comprising an integral body of strata of aluminum, aluminum oxide, and a superposed coating of a relatively more conducting solid than said intermediate oxide layer and in inactive chemical relationship with the remaining strata.

2. An electrical condenser, comprising an integral body of strata of aluminum, aluminum oxide, and a stratum including copper.

3. An electrical condenser, comprising an integral body of strata of aluminum, aluminum oxide, and a stratum including copper and a copper compound.

4. An electrical condenser, comprising an

70

75

80

85

90

95

100

105

110

115

120

125

130

- integral body of strata of aluminum, aluminum oxide, and copper overlaid with a coating of silver.
5. An electrical condenser, comprising an integral body of strata of aluminum, aluminum oxide, and copper overlaid with a coating of silver and a metal foil about the latter affording contact means thereto.
6. An electrical condenser, comprising a strip of aluminum having a projecting contact lug and its remaining surface being coated with an integral layer of aluminum oxide of minute thickness, an integral coating of copper thereof, an integral overlying coating of silver, a cover of metal foil about the latter affording a second contact, and means insulating said foil from the said contact lug.
7. A non-rectifying electrical condenser, comprising a metal foil, a dielectric coating consisting of a compound of said foil over one face thereof, molecularly associated therewith and of a thickness of the order of magnitude of  $10^{-4}$  mm., and a conductor layer over said dielectric coating and in molecular contact therewith and in inactive chemical relationships with the said metal foil and dielectric coating.
8. A non-rectifying electrical condenser, comprising a flexible metal foil, a dielectric coating consisting of a compound of said foil over one face thereof, molecularly associated therewith and of a thickness of the order of magnitude of  $10^{-4}$  mm., and a conducting layer over said dielectric coating and in molecular contact therewith and in inactive chemical relationship with the said metal foil and dielectric coating.
9. A non-rectifying electrical condenser, comprising a flexible metal foil, a dielectric coating consisting of a compound of said foil over one face thereof, molecularly associated therewith and of a thickness of the order of magnitude of  $10^{-4}$  mm., and a metallic layer over said dielectric coating and in molecular contact therewith and in inactive chemical relationship with the said metal foil and dielectric coating.
10. An electrical device embodying three molecularly associated layers, the two outer layers being conductive and in inactive chemical relationship to each other, one of said layers consisting of a filming metal, and an intermediate dielectric layer consisting of a compound of said filming metal.
11. An electrical device embodying three molecularly associated layers, the two outer layers being conductive and in inactive chemical relationship to each other, one of said layers consisting of a filming metal, an intermediate dielectric layer consisting of a compound of said filming metal, and an additional and more conductive layer over the layer opposite the filming metal layer.
12. An electrical device embodying three molecularly associated layers, the two outer layers being conductive and in inactive chemical relationship to each other, one of said layers consisting of a filming metal, an intermediate dielectric layer consisting of a compound of said filming metal, and an additional and more conductive layer over the layer opposite the filming metal layer and molecularly associated therewith.
13. An electrical device embodying three molecularly associated layers, the two outer layers being conductive and in inactive chemical relationship to each other, one of said layers consisting of a filming metal, and an intermediate dielectric layer consisting of a compound of said filming metal of substantially uniform thickness.
14. An electrical device embodying three molecularly associated layers, the two outer layers being conductive and in inactive chemical relationship to each other, one of said layers consisting of a filming metal, and an intermediate dielectric layer consisting of a compound of said filming metal, and of the order of magnitude of  $10^{-4}$  mm.
15. An electrical device embodying an integral strip of two strata of conducting solid material in inactive chemical relationship to each other and one of which is of a filming type metal, an intermediate dielectric consisting of a compound of said filming type metal stratum and of substantially uniform thickness and in inactive chemical relationship with the outer layer other than the film-forming layer, and a metal foil about one of the said strata of conducting solid materials affording contact means thereto.
16. An electrical device embodying an integral strip of two strata of conducting solid material in inactive chemical relationship to each other and one of which is of a filming type metal and one of which also has a projecting contact lug, an intermediate dielectric consisting of a compound of said filming type metal stratum and of substantially uniform thickness and in inactive chemical relationship with the outer layer other than the film-forming layer, and a metal foil about the other of the said strata of conducting solid materials affording contact means thereto.
- In testimony whereof I affix my signature.
- JULIUS EDGAR LILIENFELD.